

## UNITED STATES PATENT OFFICE.

FRANK J. FRIESE AND JOHN E. GILBERT, OF ST. LOUIS, MISSOURI,  
ASSIGNORS OF TWO-THIRDS TO EDWARD A. MORE, OF ST. LOUIS,  
MISSOURI.

## MOLD FOR MAKING BRASS CASTINGS.

SPECIFICATION forming part of Letters Patent No. 772,712, dated October 18, 1904.

Application filed March 29, 1904. Serial No. 200,656. (No model.)

*To all whom it may concern:*

Be it known that we, FRANK J. FRIESE and JOHN E. GILBERT, citizens of the United States, residing in the city of St. Louis and State of Missouri, have invented certain new and useful Improvements in Molds for Making Brass Castings, of which the following is a full, clear, and exact description.

Our present invention relates to an improved mold of the general character of that shown, described, and claimed in United States Letters Patent No. 745,005, issued November 24, 1903, to ourselves and Edward A. More, the object of our invention being the same as that mentioned in said patent—*i. e.*, to make a brass casting in a metal mold which will be smooth and perfect when produced and to furnish a mold against which the molten metal will lie smoothly and quietly. In the patent referred to the cavity of the metal mold is described and claimed as being coated with an aluminium paint. The molten brass will lie quietly against the sides of a mold of this sort, and the object molded comes out of the mold with a luster that renders further polishing unnecessary. We have found by a series of experiments that a similar result can be accomplished by mixing aluminium intimately with the iron that forms the body of the mold, the percentage of aluminium being not less than two or more than ten per cent., as less than two per cent. fails to accomplish the desired result and more than ten per cent.

results in detriment to the mold, due to the molten metal in such proportions eating into the iron mold.

In carrying out our invention we first melt the iron (that is to constitute the body of the mold) and then mix therewith from two to ten per cent. of aluminium. Our best results have been attained by adding five per cent. of aluminium to the molten iron. After the aluminium is thoroughly mixed with the iron the metal is poured into a suitable mold to form the mold for making the brass casting, and the said brass casting when produced will be found to have a smooth perfect surface and homogeneous throughout.

We claim as our invention—

1. A metallic mold for making brass castings, which is formed of an intimate mixture of iron with from two to ten per cent. of aluminium, as set forth.
2. A metallic mold for making brass castings, which is formed of an intimate mixture of iron with approximately five per cent. of aluminium, as set forth.
3. A metallic mold for making brass castings which contains iron and aluminium; the aluminium being intimately mixed with the iron throughout the mold.

FRANK J. FRIESE.  
JOHN E. GILBERT.

In presence of—

BLANCHE HOGAN,  
E. S. KNIGHT.